

1

3,511,664

### PHOTOGRAPHIC SILVER HALIDE LIGHT-SENSITIVE ELEMENT

Yoshiyuki Nakazawa, Reiichi Ohi, Hiroshi Misu, and Masanao Hinata, Kanagawa, Japan, assignors to Fuji Shashin Film Kabushiki Kaisha, Kanagawa, Japan, a corporation of Japan

No Drawing. Filed Aug. 29, 1966, Ser. No. 575,510  
Claims priority, application Japan, Aug. 30, 1965,  
40/52,488

Int. Cl. G03c 1/10

U.S. Cl. 96—104

18 Claims

#### ABSTRACT OF THE DISCLOSURE

A photographic silver halide element comprising a support and a light-sensitive emulsion containing the sensitizing dye having the general formula:



wherein R<sub>1</sub> represents a member selected from the group consisting of the following class A and the following class B.

Class A:



and



Class B: an alkyl group having less than 6 carbon atoms and an allyl group; R<sub>2</sub> represents a member selected from the above-mentioned class B; R<sub>3</sub> represents a member selected from the above-mentioned class A; and Y represents a non-metal atom necessary for completing a heterocyclic ring selected from the group consisting of thiazoles and benzothiazoles and the compound having the general formula:



wherein R<sub>4</sub> and R<sub>5</sub> each represents a member selected from the group consisting of a halogen atom, a hydroxyl group, and NH<sub>2</sub>; R<sub>6</sub> represents a member selected from the group consisting of an aryl group and aralkyl group; and R represents a member selected from the group consisting of a hydrogen atom, an alkali metal, ammonium, and an amine salt.

The present invention relates to a photographic silver halide light-sensitive element and more particularly to a photographic silver halide light-sensitive element containing a rhodacyanine sensitizing dye and having improved preservability.

It has been well known that when a sensitizing dye is incorporated in a silver halide emulsion during the production of photographic light-sensitive elements, the

2

range of the light sensitive wave length of the silver halide emulsion is enlarged and the emulsion is optically sensitized. Moreover, it has also been known that among various sensitizing dyes, a rhodacyanine sensitizing dye provides a photographic silver halide emulsion with a red sensitivity.

The rhodacyanine sensitizing dyes having the general Formula I sensitize remarkably a silver halide emulsion;



wherein R<sub>1</sub> represents a group selected from class A and class B, R<sub>2</sub> represents a group selected from class B, and R<sub>3</sub> represents a group selected from class A.

Class A:



Class B: an alkyl group having less than 6 carbon atoms and allyl group (wherein, if R<sub>1</sub> is selected from class A, —SO<sub>3</sub>H of the group may be in the state of its salt); and Y represents a non-metal atom necessary of forming a heterocyclic ring consisting of thiazoles and benzothiazoles.

Besides providing a silver halide emulsion with a high sensitivity, the sensitizing dye having above-mentioned general Formula I has such merits that in case where the sensitizing dye is present together with a water-soluble or oil-soluble coupler in an emulsion before coating, the reduction of the coupler in sensitivity is extremely less and hence a highly sensitive emulsion is obtained as compared with the case of using a sensitizing dye wherein R<sub>1</sub> and R<sub>2</sub> are alkyl groups, aralkyl groups, or alkenyl groups. Further, as the general characteristics peculiar to the rhodacyanine dye having a quinoline ring at the



position as shown in general Formula I, the light sensitive element prepared by employing such a sensitizing dye has an excellent range and position of spectral sensitive wave length suitable for the red-sensitive layer material of a multi-layer color photographic light-sensitive element. However, there is a fault that a silver halide light-sensitive element containing the sensitizing dye (I) tends to reduce its sensitivity during preservation. Accordingly, in spite of the excellent properties of the sensitizing dye (I), such a dye alone has not been practically used.

However, the above-mentioned sensitizing dye (I) may be used in some condition, that is, there is an example where such a dye is employed together with some kind of water-soluble coupler since such a coupler is considered to have a function of correcting the above-mentioned faults of the sensitizing dye.

Therefore, an object of this invention is to enable the practical use of the rhodacyanine dye shown by general Formula I in photography.

Other objects of the present invention is to provide a photographic silver halide light-sensitive element containing the rhodacyanine dye having general Formula I without accompanied with the above-mentioned fault.

Other objects and the merits of the present invention will become apparent from the following description of our invention.

These objects are accomplished according to the instant invention by incorporating in the silver halide emulsion layer containing the rhodacyanine sensitizing dye having general Formula I the compound having the general Formula II



wherein R<sub>4</sub> and R<sub>5</sub> each represents a halogen atom, a hydroxyl group or —NHR<sub>6</sub> (where, R<sub>6</sub> is an aryl group or an aralkyl group) and D is a hydrogen atom, an alkali metal, ammonium, or an amine salt.

The inventors have found that by incorporating the compound (II) the reduction in sensitivity of the photographic silver halide light-sensitive element containing the sensitizing dye (I) during preservation can be markedly prevented.

That is, it has been found that the sensitizing dye (I) the practical use of which alone is considered to be difficult in spite of the above-mentioned many merits can be used practically by incorporating in a silver halide emulsion the sensitizing dye (I) together with the compound (II) in accordance with the present invention, whereby the sensitizing dye can be effectively utilized without giving bad influences on the preservability.

The present invention will now be explained while comparing with conventional known examples.

For example, there is disclosed in Japanese Pat. 4,724/53 that a supersensitizing effect can be obtained by using the compound having the following general Formula III similar to the above-mentioned compound (II) used in our invention to a sensitizing dye.

The known compound has the general formula



wherein B and B' each represents



(where R and R' each represents a hydrogen atom, an alkyl group, an aryl group, an aralkyl group, an acyl group, an oxyalkyl group, a substituted or unsubstituted carbamyl group, a heterocyclic group or a group having a heterocyclic ring) and X and X' each represents a hydrogen atom or SO<sub>3</sub>H.

In the above-cited patent, there is no limitation about the sensitizing dye and also the scope of compound (III) is very large. However, the supersensitizing effect by the addition of compound (III) has no relation to the effect for preventing the reduction of sensitivity by the addition of compound (II), and the sensitivity-reduction preventing effect by the addition of compound (II) in accordance with the present invention can be obtained about only the sensitizing dye shown by general Formula I, that is, the addition of compound (II) is ineffective in the case of using other sensitizing dyes.

For example, among the compounds shown by general Formula III, ones most similar to the compound (II) of our invention, that is, the compound wherein B and

B' in formula (III) are a triazinyl group is illustrated by the general Formula IV.



The extent of the supersensitizing effect by the above compound is varied according to the kinds of groups R<sub>7</sub>,

R<sub>8</sub>, R<sub>9</sub> and R<sub>10</sub>. That is, among the compounds having the above Formula IV, the compound having



as R<sub>7</sub> and R<sub>9</sub> corresponds to compound (II) of our invention, and the combination of only the compound (II) and sensitizing dye (I) has the effect of preventing sensitivity reduction during preservation, which is a feature of our invention. Compound (II) of our invention has never been noticed from a view point of supersensitization, and it has never been attempted to incorporate in a silver halide emulsion the compound (II) together with a sensitizing dye. Further, a similar case to the above-cited Japanese patent is disclosed in U.S. Pat. 2,947,630 wherein a supersensitizing effect is obtained by using a rhodacyanine sensitizing dye and a compound similar to compound (II) of our invention, but as mentioned above in connection with the Japanese patent, the purpose and the effect of the U.S. patent are different from those of our invention, which can be attained by using only the specific compound and the specific sensitizing dye.

That is, as shown in below Example 3, there are compounds having an effect of preventing the sensitivity reduction of light sensitive elements during preservation and compounds showing no such action although they have a similar structure and a similar super color sensitizing power, and among the compounds (III) and the compounds similar to them, only compounds (II) have a power of preventing the reduction in sensitivity of the light-sensitive element during preservation.

It is also disclosed in British Pat. 852,074 that a compound similar to the compound (II) has a antifoggant and/or antistain action in a photographic emulsion containing a coupler. However, the reduction in sensitivity of a light sensitive element containing the sensitizing dye (I) during preservation occurs independently of the presence of coupler and the prevention of the reduction in sensitivity according to the present invention can be accomplished independently of the presence of coupler.

The known compounds described in the above-mentioned British patent are mainly aminostilbene compounds but it should be noticed that the compound (II) used in the present invention is weak soluble in water while water-soluble aminostilbene compounds cannot prevent the reduction in sensitivity of light-sensitive elements during preservation. Further, an aminostilbene compound has been known as a fluorescent whitening agent and when it is used in photographic light-sensitive elements, in particular, it is used in a large proportion, the reflection density (maximum density) of an image of the photographic light sensitive element after processing is reduced by the

fluorescence in the image layer caused by the compound and moreover, when it is employed in color photographic light-sensitive elements (such as color photographic papers and the like), the reduction in reflection density of the yellow image is remarkable.

However, these drawbacks are removed by using the 5

weak-soluble compound (II) of the present invention since the fluorescence thereof in the image layer is very weak.

Listed below are representative compounds selected from those represented by Formula I, although our invention is not limited in any sense to these particular compounds.



(I-8)



As the examples of the compound having general Formula II used in this invention, there are illustrated as follows:

(II-1)



(II-2)



(II-3)



(II-4)



(II-5)



A suitable density of the sensitizing dye (I) of this invention in a silver halide emulsion is 0.002 to 0.2 g. per mol of silver halide and that of the compound (II) is 0.05 to 1 g. per mol of silver halide, and the ratio of the sensitizing dye (I) to compound (II) is suitably from 1:2 to 1:200, in particular from 1:10 to 1:60.

The sensitizing dye (I) may be added in a silver halide emulsion in a manner well known in the field. The com-

ound (II) may be added in a silver halide emulsion as a solution of an organic solvent such as methanol and ethanol. The addition of the sensitizing dye (I) and

70

the compound (II) is conducted prior to coating. The sensitizing dye (I) may be added in a silver halide emulsion before or after or together with the compound (II).

For the silver halide emulsion in this invention may be used various silver salts, such as, silver chloride, silver bromide, silver iodide, silver iodo-bromide, silver chloro-bromide or silver chloro-iodo-bromide and also the silver halide emulsion may contain such usual addi-

tives as, a chemical sensitizer, a hardening agent, an anti-fogging agent, a wetting agent, a stabilizer, a plasticizer, a developing accelerator, and a anti-bronzing agent as well as a coupler capable of forming a cyan image by color development.

The silver halide emulsion may be applied by a suitable manner to a suitable support such as a glass plate, a film of a cellulose derivative, a film of a synthetic resin or a baryta paper.

The following are examples of the present invention.

### EXAMPLE 1

A silver chloro-bromide emulsion (chloride:bromide=60 moles:40 moles) containing the sensitizing dye (I) was applied to a film base of cellulose acetate. Apart from this, the same silver halide emulsion containing the sensitizing dye (I) together with the compound (II) was applied to a film base of cellulose acetate. Thus prepared light sensitive films were measured about the sensitivities directly after coating and after preserved for a long period of time and the change of the sensitivities are shown in Table 2.

The sensitivity was shown by the red sensitivity obtained by exposing through Fuji-7 Filter (transmitting the light having longer wave lengths than 590 millimicrons. The sample was preserved for 180 days at a temperature of 23° C. and at a relative humidity of 60%. The development was conducted for 6 minutes using the developer showing in Table 1. The sensitivity value was shown by log E (where E is the exposure amount necessary for providing fog+optical density being 0.1). The sensitivity change by preservation ( $\Delta \log E$ ) was shown by a value of log E directly after coating subtracted by the value of log E after preservation.

TABLE 1.—COMPOSITION OF DEVELOPER

|                                   | G.  |
|-----------------------------------|-----|
| N-methyl-para-aminophenol sulfate | 2.0 |
| Hydroquinone                      | 4.0 |
| Sodium sulfite                    | 40  |
| Sodium carbonate (mono-hydrate)   | 28  |
| Potassium bromide                 | 1   |
| Water to make 1 liter.            |     |

TABLE 2

| Sensitizing dye (I) (mg./gram<br>molecule of silver halide) | Compound (II)<br>(mg./gram<br>molecule of<br>silver halide) | $\Delta \log E$ | Change<br>in fog |
|-------------------------------------------------------------|-------------------------------------------------------------|-----------------|------------------|
| (a) I-1 (30)                                                | None                                                        | -0.27           | +0.01            |
| (b) I-1 (30)                                                | II-1 (500)                                                  | -0.05           | +0.01            |
| (c) I-1 (50)                                                | None                                                        | -0.34           | +0.05            |
| (d) I-1 (50)                                                | II-1 (800)                                                  | -0.11           | +0.05            |
| (e) I-2 (100)                                               | None                                                        | -0.25           | +0.00            |
| (f) I-2 (100)                                               | II-1 (500)                                                  | -0.03           | +0.00            |
| (g) I-3 (25)                                                | None                                                        | -0.27           | +0.01            |
| (h) I-3 (25)                                                | II-2 (500)                                                  | -0.07           | +0.01            |
| (i) I-4 (40)                                                | None                                                        | -0.30           | +0.01            |
| (j) I-4 (40)                                                | II-3 (1,000)                                                | -0.12           | +0.01            |

From the results shown in Table 2, it is clear that the change insensitivity of the light-sensitive element after

5  
10

### EXAMPLE 2

A photographic emulsion containing the sensitizing dye (I) and a dispersion of the coupler having the following structure



15  
20  
25  
30  
35  
40  
45  
50  
55

was applied to a baryta paper. Apart from this, a photographic emulsion containing the sensitizing dye (I), the coupler dispersion same as above, and the compound (II) was applied to a baryta paper similarly.

The sensitivity change of the both types of thus prepared light-sensitive papers was measured between the ones directly after coating and ones after preservation, the results of which are shown in Table 4.

The filter for exposure and the preservative conditions were same as in Example 1. The development was conducted for 9 minutes at 20° C. in the developer shown in Table 3. Thus developed photographic paper was, rinsed with water, fixed, bleached, and then rinsed with water. The sensitivity value was indicated by log E (E is an exposure amount necessary for giving fog+optical density being 0.1). The change in sensitivity by preservation was shown by  $\Delta \log E$ .

TABLE 3.—COMPOSITION OF DEVELOPER

|                                                                        | G.  |
|------------------------------------------------------------------------|-----|
| Sodium sulfite (anhydrous)                                             | 2.0 |
| N-ethyl-N-( $\beta$ -hydroxyethyl) - para-phenylenediamine-semihydrate | 4.0 |
| Sodium carbonate (mono-hydrate)                                        | 60  |
| Potassium bromide                                                      | 1.0 |
| Hydroxylamine sulfate                                                  | 2.4 |
| Water to make 1 liter.                                                 |     |

TABLE 4

| Sensitizing dye (I)<br>(mg./gram<br>molecule of<br>silver halide) | Compound (II)<br>(mg./gram<br>molecule of<br>silver halide) | Change<br>in fog |
|-------------------------------------------------------------------|-------------------------------------------------------------|------------------|
| (a) I-5 (25)                                                      | None                                                        | -0.29            |
| (b) I-5 (25)                                                      | II-1 (800)                                                  | -0.07            |
| (c) I-6 (30)                                                      | None                                                        | -0.21            |
| (d) I-6 (30)                                                      | II-1 (500)                                                  | -0.04            |
| (e) I-7 (30)                                                      | None                                                        | -0.18            |
| (f) I-7 (30)                                                      | II-3 (800)                                                  | -0.05            |
| (g) I-8 (10)                                                      | None                                                        | -0.15            |
| (h) I-8 (10)                                                      | II-4 (180)                                                  | -0.02            |

### EXAMPLE 3

Each of a photographic emulsion (a) containing the coupler dispersion as in Example 2 and the sensitizing dye (I), a photographic emulsion (b) containing the coupler dispersion, the sensitizing dye (I) and the compound (II) and a photographic emulsion (c) containing the coupler dispersion, the sensitizing dye (I) and the compound having the following general Formula V was applied to a baryta paper followed by drying,



(V)

preservation is remarkably reduced by incorporating the compound (II) together with the sensitizing dye (I).

75  
and thereafter, the sensitivity change of them between one directly after coating and one after preservation was

measured by the same conditions as in Example 2, the results of which are shown in Table 5.

TABLE 5

| Sensitizing dye<br>(mg./gram<br>molecule of<br>silver halide) | Compound<br>(mg./gram<br>molecule of<br>silver halide) | Relative<br>sensi-<br>tivity | $\Delta \log E$ | Change<br>in fog | 5 |
|---------------------------------------------------------------|--------------------------------------------------------|------------------------------|-----------------|------------------|---|
| (a) I-3 (25)                                                  | None                                                   | 100                          | -0.25           | +0.01            |   |
| (b) I-3 (25)                                                  | II-1 (500)                                             | 230                          | -0.07           | +0.01            |   |
| (c) I-3 (25)                                                  | V (500)                                                | 235                          | -0.26           | +0.01            |   |



The control compound (V) as mentioned above is one of the compound (III) having a super sensitizing effect and the structure thereof is very similar to that of the compound (II) used in the present invention but the compound showed no effect for preventing the reduction in sensitivity by preservation. 20

What is claimed is:

1. A photographic silver halide element comprising a support and a silver halide light-sensitive emulsion containing a sensitizing dye having the general formula:



wherein R1 represents a member selected from the group consisting of the following class A and the following class B;

Class A:



Class B: an alkyl group having less than six carbon atoms and an allyl group; R2 represents a member selected from the above-mentioned class B; R3 represents a member selected from the above-mentioned class A; and Y represents a non-metal atom necessary for completing a heterocyclic ring selected from the group consisting of thiazoles and benzothiazoles and a compound having the general formula:



wherein R4 and R5 each represents a member selected from the group consisting of a halogen atom, a hydroxyl group, and  $\text{NHR}_6$ ; R6 represents a member selected from the group consisting of an aryl group and an aralkyl group; and D represents a member selected from the group consisting of a hydrogen atom, an alkali metal, ammonium, and an amine salt.

2. The photographic silver halide element according to claim 1 wherein the proportion of said sensitizing dye in the silver halide light-sensitive emulsion is 0.002-0.2 g. per mol of the silver halide in the emulsion.

3. The photographic silver halide element according to claim 1 wherein the proportion of said compound in the silver halide light-sensitive emulsion is 0.05-1 g. per mol of the silver halide in the emulsion.

4. The photographic silver halide element according to claim 1 wherein the proportion ratio of said sensitizing dye to said compound is from 1:2 to 1:200, preferably from 1:10 to 1:60.

5. The photographic silver halide element according to claim 1 wherein said emulsion layer contains a cyan coupler.

6. The photographic silver halide element according to claim 1, wherein said sensitizing dye is



7. The photographic silver halide element according to claim 1 wherein said sensitizing dye is



8. The photographic silver halide element according to claim 1 wherein said sensitizing dye is

(I-3)



9. The photographic silver halide element according to claim 1 wherein said sensitizing dye is

(I-4)



10. The photographic silver halide element according to claim 1 wherein said sensitizing dye is

(I-5)



11. The photographic silver halide element according to claim 1 wherein said sensitizing dye is

(I-6)



12. The photographic silver halide element according to claim 1 wherein said sensitizing dye is

(I-7)



13. The photographic silver halide element according to claim 1 wherein said sensitizing dye is

(I-8)



14. The photographic silver halide element according to claim 1 wherein said compound is

(II-1)



15. The photographic silver halide element according to claim 1 wherein said compound is

(II-2)



16. The photographic silver halide element according to claim 1 wherein said compound is

(II-3)



17. The photographic silver halide element according to claim 1 wherein said compound is

(II-4)



18. The photographic silver halide element according to claim 1 wherein said compound is

(II-5)



#### References Cited

#### UNITED STATES PATENTS

2,947,630 8/1960 Jones 96—105

#### FOREIGN PATENTS

4,724 1953 Japan.  
852,074 10/1960 Great Britain.

#### OTHER REFERENCES

Fiat Report No. 943, pp. 53-56.

NORMAN G. TORCHIN, Primary Examiner

M. F. KELLEY, Assistant Examiner

U.S. CL. X.R.

96—109, 127